

Oct. 29, 1940.

B. GASPAR

2,219,306

PHOTOGRAPHIC MATERIAL

Filed Dec. 3, 1938



Inventor

Bela Gaspar

By

F. Gerald Goye

Attorney

## UNITED STATES PATENT OFFICE

2,219,306

## PHOTOGRAPHIC MATERIAL

Béla Gáspár, Hollywood, Calif.

Application December 3, 1938, Serial No. 243,890  
In Great Britain December 9, 1937

6 Claims.

(Cl. 95—2)

The present invention relates to a photographic multilayer material for color photographic purposes. Some or all of the various light sensitive layers contain, already before the exposure, the dye necessary for the formation of the final image. As is known, such light-sensitive materials after exposure of the light sensitive layers, are converted into colored pictures by means of local removal of the dyestuff. If two or more layers are arranged upon the same support, it is necessary to sensitize at least two of the layers for differently colored light in order to produce the desired color selection picture in each individual layer with light corresponding to the sensitivity.

Now it is known, that an ordinary silver bromide emulsion is sensitive to blue light and remains so even if a predominant sensitivity to green, red or infrared is imparted to the emulsion by the addition of a special color sensitizer. For this reason in a multilayer material composed of two or more silver halide layers at least one specially sensitized layer is sensitive not only to the light for which the layer is predominantly sensitized, but also to blue light. For an analogous reason two emulsions are sensitive to green light, if the one contains a sensitizer for green and if the other one contains a panchromatic sensitizer or one which imparts a predominant sensitivity to red but in addition a noticeable sensitivity to green.

The sensitivity of two superimposed layers to the same light renders a correct color separation very difficult and it is an object of the present invention to restrict the action of light to that of the two layers which is first hit by the light falling upon the composite layers. In a predyed multilayer material of the kind described, in which at least one light sensitive layer is sensitive not only to light for which the layer is predominantly sensitive but also to light for which a superimposed light sensitive layer is to be exposed, the superimposed layer is, according to the present invention, dyed by a mixture of two different dyestuffs of a color complementary to the sensitivity of this layer. The one of the dyestuffs used for this purpose is resistant to the ordinary photographic treating solutions but capable of being selectively destroyed in proportion to the exposure or the silver image. The other dyestuff has substantially the same color but is easily removable by photographic treating solutions which do not remove the first named dyestuff. This first named dyestuff is used in a concentration which corresponds to the color in-

tensity necessary or desired for reproducing the most intensely colored parts of the image. The removable dyestuff is used in such a concentration that the absorption of both dyestuffs together is sufficient for preventing any light of complementary color from entering the second layer.

Instead of coloring the superposed layer as a whole by a mixture of the two dyestuffs, the auxiliary dyestuff may also be applied to the rear surface of the superposed layer or may be incorporated into an intermediate layer between the two layers in question. In this case, therefore, the layer first hit by the light is dyed by a dyestuff resistant to the ordinary photographic treating solutions and of a color complementary to the color of the light to which this layer is sensitized, the dyestuff concentration in the layer corresponding to the color intensity required at the most intensely colored points of the image.

The properties of the layer allow the incident light to enter the colored layer and to penetrate it where the intensity has its maximum value. The penetrating light, however, is absorbed at the rear surface or in the intermediate layer by the auxiliary dyestuff and thus the light-sensitive layer behind is effectively screened.

*Example.*—Referring to the drawing, on a paper support there are coated in superposition a blue-green emulsion sensitized to red light, a magenta dyed emulsion sensitized to green and a yellow dyed blue-sensitive emulsion.

The yellow dyed emulsion is the top layer and contains the dyestuff Xylenewalkgelb G (Shultz Farbstofftabellen, volume 2) in the form of its calcium salt in a concentration of 0.45 g. per sq. m. The same layer or a separate layer of plain gelatine arranged behind the same contains 1 to 2 g. per sq. m. of the dyestuff 4,4'-methylene-bis-1-(p-sulphophenyl)-3-methyl-pyrazolone-5 in the form of its triphenylguanidine salt.

A magenta layer then follows which contains 0.3 g. per sq. m. of Tuchechtbrillantrot 2B (a dyestuff supplied by the Gesellschaft fuer Chemische Industrie in Basle and similar to the dyestuff Polarbrillantrot B described in Brunner, Analyse der Azofarbstoffe, Berlin 1929, page 113) in the form of its N-methyl-naphthoquinolinium salt, which may conveniently be formed by the action of a solution containing N-methyl-quinolinium-methyl sulphonate on the dyestuff. The layer is formed by an ordinary blue-sensitive emulsion sensitized to green light by any suitable green-sensitizer, and a magenta dyestuff, such as the

sulphonic acid derived from methenyl-bis-oxy-thionaphthene or the red dyestuff obtained from 1-(p-sulpho-phenyl)-3-methyl-pyrazolone-5 and  $\beta$ -anilino-acroleine-anile as described in Example 5 of my application Ser. No. 240,860 filed Nov. 16, 1938, in the form of the diphenyl- or triphenyl- guanidine salts (which may be prepared by the action of diphenyl or triphenylguanidine acetate on the dyestuff) is present in the layer itself or in 10 a separate layer of gelatin between the magenta layer and the next layer which is a panchromatic silver bromide emulsion layer dyed by the dyestuff Pontamine Sky Blue 5BX (Schultz Farbstofftabellen, 1931, 7th ed. vol. 1. No. 513). The dyestuff 15 is used in a concentration of about 0.35 g. per sq. m. emulsion and the layer is applied to the paper support. The dyestuff 4,4'-methenyl-bis-[1-(p-sulphophenyl)-3-methyl-pyrazolone-5] and other suitable decolorisable dyestuffs are 20 described in my application Ser. 240,860 filed Nov. 16, 1938. The material may be exposed behind colored or black and white positive part images or behind a multi-color master-positive of the additive or subtractive type. The auxiliary 25 dyestuffs are decolorised after exposure of the three layer material preferably by a developer of alkaline reaction and the image-forming dyestuffs are locally destroyed after development of the silver images, for example, by an acid thiocarbamide solution or by a solution containing 30 5% hydrobromic acid. If necessary the silver is afterwards removed from the dyestuff image thus obtained.

What is claimed is:

1. A multilayer light-sensitive material, comprising a support carrying a plurality of superposed silver halide emulsion layers sensitive to light of different colors, at least one of the layers being dyed by a dye which is fast to ordinary photographic treating solutions but capable of being locally bleached in the presence of a metallic silver image and which absorbs the total spectral range of light rays for which the layer is predominantly sensitized, a second one of said plurality of superposed light-sensitive layers arranged behind said fast dyed layer being transmittant for and sensitive to such light, and a filter dye of substantially the same color as said fast dye being present in a layer in front of the said second layer but not in front of said fast dyed layer, said filter dye being removable by an agent which does not remove said fast dye.
2. A multilayer light-sensitive material, comprising a support carrying a plurality of superposed silver halide emulsion layers sensitive to light of different colors, at least one of the layers being dyed by a dye which is fast to ordinary photographic treating solutions but capable of being locally bleached in the presence of a metallic silver image and which absorbs the total spectral range of light rays for which the layer is predominantly sensitized, a second one of said plurality of superposed light-sensitive layers arranged behind said fast dyed layer being transmittant for and sensitive to such light, and a filter dye of substantially the same color as said fast dye being present in a colloid layer arranged between said fast dyed layer and said second light-sensitive layer, said filter dye being removable by an agent which does not remove said fast dye.
3. A multilayer light-sensitive material, comprising a support carrying a plurality of superposed silver halide emulsion layers sensitive to

light of different colors, at least one of the layers being dyed by a dye which is fast to ordinary photographic treating solutions but capable of being locally bleached in the presence of a metallic silver image and which absorbs the total spectral range of light rays for which the layer is predominantly sensitized, a second one of said plurality of superposed light-sensitive layers arranged behind said fast dyed layer being transmittant for and sensitive to such light, and a filter dye of substantially the same color as said fast dye being present in the said fast dyed light-sensitive emulsion layer, said filter dye being removable by an agent which does not remove said fast dye. 15

4. A multilayer light-sensitive material, comprising a support carrying a plurality of superposed silver halide emulsion layers sensitive to light of different colors, at least one of the layers being dyed by a dye which is fast to ordinary photographic treating solutions but capable of being locally bleached in the presence of a metallic silver image and which absorbs the total spectral range of light rays for which the layer is predominantly sensitized, a second one of said plurality of superposed light-sensitive layers arranged behind said fast dyed layer being transmittant for and sensitive to such light, and a filter dye of substantially the same color as said fast dye and which is capable of being destroyed 30 by a photographic developer which does not remove the said fast dye, said filter dye being present in a layer in front of the said second layer but not in front of the said fast dyed layer. 35

5. A multilayer light-sensitive material, comprising a support carrying a plurality of superposed silver halide emulsion layers sensitive to light of different colors, at least one of the layers being dyed by a dye which is fast to ordinary photographic treating solutions but capable of being locally bleached in the presence of a metallic silver image and which absorbs the total spectral range of light rays for which the layer is predominantly sensitized, a second one of said plurality of superposed light-sensitive layers arranged behind said fast dyed layer being transmittant for and sensitive to such light, and a filter dye of substantially the same color as said fast dye being present in a layer in front of the said second layer but not in front of said fast dyed layer, the absorption of said filter dye being greater than the absorption of said fast dye and said filter dye being removable by an agent which does not remove said fast dye. 40 45 50

6. A multilayer light-sensitive material, comprising a support carrying a plurality of superposed silver halide emulsion layers sensitive to light of different colors, at least one of the layers being dyed by a dye which is fast to ordinary photographic treating solutions but capable of being locally bleached in the presence of a metallic silver image and which absorbs the total spectral range of light rays for which the layer is predominantly sensitized, a second one of said plurality of superposed light-sensitive layers arranged behind said fast dyed layer being transmittant for and sensitive to such light, and a filter dye of substantially the same color as said fast dye being present in the said fast dyed light-sensitive emulsion layer, the absorption of said filter dye being greater than the absorption of said fast dye and said filter dye being removable by an agent which does not remove said fast dye. 60 65 70

BÉLA GÁSPÁR.